

X 20074

United S

3,644,597

Entd Feb. 22, 1972

## 1

3,644,597

REACTION PRODUCT OF 2,3-DIBROMOPROPANOL  
AND PHOSPHORUS PENTOXIDEAbraham S. Endler, Flushing, N.Y., assignor to Apex  
Chemical Co., Inc., Elizabethport, N.J.  
No Drawing. Filed Jan. 28, 1969, Ser. No. 794,805  
Int. Cl. C07f 9/08; C09k 3/28

U.S. CL. 260—933

9 Claims

## ABSTRACT OF THE DISCLOSURE

The product of the reaction of 2,3-dibromopropanol, phosphorus pentoxide in an amount sufficient to provide therefrom 1 to 2 atoms of phosphorus per molecule of 2,3-dibromopropanol, either additional phosphorus pentoxide, phosphoric acid or polyphosphoric acid in an amount to provide, with the first mentioned phosphorus pentoxide, a total of 3 to 25 atoms of phosphorus per molecule of 2,3-dibromopropanol and sufficient free water, if necessary, to provide, with any combined water that may be present, a water content of 0.8 molecule thereof for each phosphorus atom in the additional phosphorus pentoxide, the phosphoric acid or the polyphosphoric acid, is dissolved in water with sufficient ammonia to adjust the pH of the resulting solution to within the range from 5 to 8, whereby to provide a water-soluble flame retardant for textile fibers or fabrics. The reaction mixture may further include a maximum of 1 molecule of urea for each 2 atoms of phosphorus in the total number of the latter. The solution for imparting flame retarding properties to textile materials may include a fire retardant salt, such as ammonium phosphate, along with the stated reaction product provided that the latter constitutes at least 10 wt. percent of the total solids content of the solution.

This invention relates generally to flame retardants for application to textile fibers or fabrics, which are hereinafter generally referred to as textile materials, and more particularly to water-soluble, organic flame retardants.

A number of ammonium salts of inorganic acids are known to be effective as flame retardants when applied in sufficient proportion to textile fabrics. One general disadvantage of all of these salts is that they tend to crystallize on the surface of the textile fibers, or internally, creating either undesirable stiffness or an undesirable whitish powdery surface appearance.

Many organic salts do not crystallize in this manner, and do not cause these undesirable effects, but unfortunately organic salts in general do not exhibit any flame retardant action. Ammonium salts of alkyl acid esters of phosphoric acid show a slight flame retardant action on cellulosic fibers, provided that the alkyl groups in the ester do not contain excessive proportions of carbon and hydrogen. Thus, partial esters of phosphoric acid with ethylene glycol, glycerol, and other glycols are known to have some desirable fire retardant properties. Unfortunately a much higher weight percent add-on of these esters is needed than with the common inorganic fire retardant salts, such as ammonium phosphate.

The use, as a flame retardant, of the ammonium salt of the ester of 2,3-dibromopropanol with phosphoric acid, that is, the ammonium salt of 2,3-dibromopropylphosphoric ester, has been disclosed in prior literature. Although such compound is an effective flame retardant and does not crystallize either on the surface of the treated textile fibers, or internally therein, it is relatively costly, as compared with ammonium phosphate or ammonium sulfamate, by reason of the high cost of the 2,3-

## 2

dibromopropanol constituting the major proportion thereof, and further it is disadvantageously characterized by a sticky or tacky feel and a brownish color. The reported ammonium salt of 2,3-dibromopropylphosphoric ester is also only sparingly soluble in water which leads to difficulties in its application, as a flame retardant, to textile fibers or fabrics.

Accordingly, it is an object of this invention to provide relatively low-cost flame retardants of almost water-white color that can be applied to a wide variety of textile materials, either in the form of fibers or fabrics, to afford thereto effective flame-retarding properties without unduly affecting the feel of the fabric and without crystallizing or otherwise contributing to an undesirable appearance of the fabric.

A further object is to provide flame retardants having the foregoing characteristics and which are water-soluble for ease of application to textile materials.

Still another object is to provide flame retardants that are as effective as the mentioned ammonium salt of 2,3-dibromopropylphosphoric ester and similarly do not crystallize, but which are free of the undesirable characteristics of the known compound, that is, the tacky feel, brownish color and poor solubility in water of the latter.

In accordance with this invention, the foregoing objects are achieved by reacting 2,3-dibromopropanol with phosphorus pentoxide in an amount sufficient to provide at least 1 atom of phosphorus in such phosphorus pentoxide per molecule of 2,3-dibromopropanol, and with either additional phosphorus pentoxide, phosphoric acid or polyphosphoric acid in an amount sufficient to provide, with the first mentioned phosphorus pentoxide, at least 3 atoms of phosphorus per molecule of 2,3-dibromopropanol, the water content of the reaction mixture being adjusted to provide approximately 0.8 molecule of combined and/or free water for each phosphorus atom in the additional phosphorus pentoxide, phosphoric acid or polyphosphoric acid, and by dissolving the resulting reaction product in water with sufficient ammonia to adjust the pH of the solution to within the range from 5 to 8.

Where the 2,3-dibromopropanol is reacted with phosphorus pentoxide and 115% polyphosphoric acid (also known as triphosphoric acid) the latter has 0.8 molecule of combined water per atom of phosphorus therein, so that no adjustment of the water content of the reaction mixture is required. Where the 2,3-dibromopropanol is reacted only with phosphorus pentoxide, free water is added to the reaction mixture to provide the 0.8 molecule of water per atom of phosphorus in the phosphorus pentoxide employed in excess of that required to furnish at least 1 atom of phosphorus per molecule of 2,3-dibromopropanol. Where the 2,3-dibromopropanol is reacted with phosphorus pentoxide and 85% phosphoric acid, which contains 15%, by weight, of free water and further 1.5 molecules of combined water per atom of phosphorus in the phosphoric acid, the necessary adjustment of the total water content of the reaction mixture can be achieved by employing partly phosphorus pentoxide, which has no combined water, and partly 85% phosphoric acid to provide the phosphorus atoms in excess of the phosphorus atoms furnished in the form of phosphorus pentoxide to make available at least 1 atom of phosphorus for each molecule of 2,3-dibromopropanol. Similarly, where the reaction mixture contains 2,3-dibromopropanol, phosphorus pentoxide and 105% polyphosphoric acid, which is also known as superphosphoric acid and contains 1.23 molecules of combined water per atom of phosphorus therein, the necessary adjustment of the water content is effected by employing an excess of phosphorus pentoxide beyond that required to provide at least 1 atom of phosphorus per molecule of 2,3-dibromopropanol.

Although the above general description of the reaction

mixture according to this invention states that the amount of phosphorus pentoxide provided therein, in the first instance, is sufficient to provide at least 1 atom of phosphorus per molecule of 2,3-dibromopropanol in the reaction mixture, the amount of phosphorus pentoxide included for the foregoing purpose preferably should not exceed that which provides 2 atoms of phosphorus (in the form of phosphorus pentoxide) per molecule of 2,3-dibromopropanol, as excessive amounts of phosphorus in the form of phosphorus pentoxide will lead to undesirable darkening of the reaction product. Of course, the foregoing limitation on the maximum amount of phosphorus pentoxide in the reaction mixture only applies to that provided for furnishing phosphorus in the form of phosphorus pentoxide and not to the phosphorus pentoxide that may be included in the reaction mixture with free water to provide the equivalent of 115% polyphosphoric acid, nor to the phosphorus pentoxide that may be employed with phosphoric acid or with 105% polyphosphoric acid to adjust the water content to the equivalent of 115% polyphosphoric acid (that is, 0.8 molecule of water per atom of phosphorus).

If the amount of phosphorus pentoxide in the reaction mixture is less than that required to provide 1 atom of phosphorus in the form of phosphorus pentoxide per molecule of 2,3-dibromopropanol, as specified above, the reaction will not be complete.

Further, although the total number of phosphorus atoms, provided in the form of phosphorus pentoxide and otherwise, may substantially exceed 3 atoms of phosphorus per molecule of 2,3-dibromopropanol, preferably no more than 25 atoms of total phosphorus per molecule of 2,3-dibromopropanol are included in the reaction mixture. Beyond the foregoing maximum ratio of phosphorus atoms to 2,3-dibromopropanol molecules in the reaction mixture, the flame retardants produced therefrom have an increased tendency to crystallize when applied to textile fibers or fabrics and the advantages inherent in the organic nature of the product are diminished.

The amount of water in which the described reaction product is dissolved is selected to preferably provide the resulting solution with solids content of the reaction product that is preferably in the range from about 50 to 55 wt. percent.

Such solution with ammonia added thereto sufficient to adjust the pH to within the range from 5 to 8, is readily soluble or dilutable with further water for application to a wide variety of textile fibers or fabrics so as to impart flame retarding properties thereto with a dry add-on of the product of this invention in the range from 3 to 30% based on the weight of fiber or fabric.

The reaction mixture from which products according to this invention result may further include urea in limited amounts that do not exceed 1 molecule of urea for each 2 atoms of the total phosphorus atoms provided in the reaction mixture. The inclusion of urea in the reaction mixture is found to improve the color of the reaction product and also to further reduce the tackiness of the dried flame retardant on the textile fibers or fabrics. However, similar desirable characteristics can be achieved without urea in the reaction mixture if the reaction temperature is carefully controlled, for example, so as to be maintained in the range between about 80 and 100° C.

The flame retardants according to this invention may be applied alone to textile materials, as previously indicated, or in admixture with one or more inorganic salts, such as, ammonium phosphate, ammonium bromide, ammonium sulfamate, ammonium sulfate and ammonium chloride, so as to substantially improve the properties of the finish imparted by the inorganic salts. The mentioned inorganic flameproofing salts tend to form whitish, powdery surface deposits when applied in amounts sufficient to impart substantial flame retarding properties to textile materials. The foregoing is particularly noted in the case of the treatment of textile fibers or fabrics which

do not readily absorb water, such as nylon, polyester, spandex, triacetate and other so-called hydrophobic fibers. However, if even such hydrophobic fibers, or textile fabrics made therefrom, are treated with mixtures of one or more of the inorganic salts, such as, ammonium phosphate, ammonium bromide, ammonium sulfamate, ammonium sulfate or ammonium chloride, and a water-soluble flame retardant according to this invention which constitutes at least 10 wt. percent of the total solids, the crystalline powdery appearance of the treated fabric is substantially eliminated, and the tendency of the inorganic salts to become dislodged from the fabric by shaking or rubbing is also greatly reduced.

An important advantage of the flame retardants according to this invention is that they exhibit the mentioned desirable properties when applied to a wide variety of textile fibers and to woven, knitted or non-woven fabrics produced from such fibers. Thus, in addition to fabrics of the previously mentioned hydrophobic fibers, the fire retardants according to this invention may be advantageously applied, either alone or in admixture with inorganic salts, to fabrics of cotton, rayon, cellulose acetate and blends thereof either with each other or with the named hydrophobic fibers.

The invention will now be further described with reference to the following specific examples which are merely illustrative:

#### EXAMPLE 1

218 grams of 2,3-dibromopropanol (1 gram-molecular weight) are disposed in a flask equipped with a stirrer and thermometer, and 172 grams of 115% polyphosphoric acid (containing 2 gram-atomic weights of phosphorus) are added to the 2,3-dibromopropanol. The contents of the flask are mixed for 15 minutes while cooling the flask contents with an external water bath, as required, to prevent a temperature rise above 80° C., whereupon, over a period of 30 minutes, 71 grams of phosphorus pentoxide (containing 1 gram-atomic weight of phosphorus) are added portionwise to the flask contents while external cooling is continued, as required, to maintain the reaction mixture temperature between 80 and 90° C. After all of the phosphorus pentoxide has been added, the reaction mixture is further stirred for 2 hours at a temperature between 80 and 90° C., and at the end of such time all of the phosphorus pentoxide has dissolved and the resulting product is a clear amber liquid.

In the above described reaction mixture, there is 1 atom of phosphorus in the form of phosphorus pentoxide per molecule of 2,3-dibromopropanol, and 2 atoms of phosphorus in the 115% polyphosphoric acid per molecule of 2,3-dibromopropanol, that is, a total of 3 atoms of phosphorus per molecule of 2,3-dibromopropanol. Further, the only water in the reaction mixture is the combined water in the 115% polyphosphoric acid which is present in the ratio of 0.8 molecule of water per atom of phosphorus in the polyphosphoric acid.

The reaction product in the form of a clear amber liquid is poured onto one-half its own weight of crushed ice, and aqua ammonia is slowly mixed in until the pH of the mixture is between 5 and 8. The resulting liquid is found to have between 50 and 55 wt. percent solids dissolved therein.

#### EXAMPLE 2

218 grams of 2,3-dibromopropanol (1 gram-molecular weight) and 516 grams of 115% polyphosphoric acid (containing 6 gram-atomic weights of phosphorus) are mixed together in a flask equipped with a stirrer and thermometer. After mixing for 10 minutes, during which time the temperature of the flask contents rises to about 40° C. and the dibromopropanol dissolves completely in the polyphosphoric acid, 180 grams of urea (3 gram-molecular weights) are added to the flask contents and the latter are warmed to 100° C. and mixed at the latter temperature for 15 minutes to completely dissolve the urea. There-

upon, 142 grams of phosphorus pentoxide (containing 2 gram-atomic weights of phosphorus) are added portionwise to the flask contents over a period of 30 minutes, with the temperature being maintained between 100 and 110° C. during such addition. The reaction mixture is then stirred for 1 hour at a temperature between 100 and 110° C., whereupon, the reaction product is poured onto one-half its weight of crushed ice and concentrated aqua ammonia is added slowly with mixing until the pH of the resulting solution is adjusted to within the range from 5 to 8. The final solution is almost colorless and somewhat turbid with a solids content of about 50 wt. percent, but an almost clear solution results when it is further diluted with water.

In the reaction mixture described in this example, there are 2 atoms of phosphorus in the form of phosphorus pentoxide per molecule of 2,3-dibromopropanol, a total of 8 atoms of phosphorus per molecule of 2,3-dibromopropanol, and the only water content is the combined water of the 115% polyphosphoric acid which is thus present in the ratio of 0.8 molecule of water per atom of phosphorus in the 115% polyphosphoric acid. Further, the urea is present in the reaction mixture in the ratio of 3 molecules of urea to 8 atoms of phosphorus.

#### EXAMPLE 3

Using a procedure similar to that of Example 2, 218 grams of 2,3-dibromopropanol (1 gram-molecular weight) are reacted with 1548 grams of 115% polyphosphoric acid (containing 18 gram atomic weights of phosphorus) and then with 120 grams of urea (2 gram-molecular weights) and finally with 142 grams of phosphorus pentoxide (2 gram-atomic weights of phosphorus).

Such reaction mixture is seen to contain 2 atoms of phosphorus in the form of phosphorus pentoxide per molecule of 2,3-dibromopropanol, a total of 20 atoms of phosphorus per molecule of 2,3-dibromopropanol, and only 2 molecules of urea for 20 total atoms of phosphorus. Further, since the only water is that present as combined water in the 115% polyphosphoric acid, there are 0.8 molecule of water for each atom of phosphorus present as the polyphosphoric acid.

The product of the above reaction mixture is mixed with crushed ice and concentrated aqua ammonia to provide a final product which is a substantially clear liquid having a pH between 5 and 8 and a solids content of about 50 wt. percent. Such liquid is further dilutable with water to yield a clear solution.

#### EXAMPLE 4

218 grams of 2,3-dibromopropanol (1 gram-molecular weight) are mixed in a flask having a stirrer and thermometer with 115.5 grams of 85% phosphoric acid (containing 1 gram-molecular weight of 100% phosphoric acid, which supplies 1 gram-atomic weight of phosphorus, and 0.94 gram-molecular weights of free water in addition to the 1.5 gram-molecular weights of water provided as combined water in the 100% phosphoric acid). Using external cooling as needed to maintain the temperature of the flask contents at 80 to 90° C., there are added, in portions, to the flask contents 213 grams of phosphorus pentoxide (representing 1½ gram-molecular weights which contain 3 gram-atomic weights of phosphorus). After one-half of the mentioned quantity of phosphorus pentoxide has been added, the mixture is stirred for 1 hour so as to dissolve all of the previously added phosphorus pentoxide. Then 120 grams of urea (2 gram-molecular weights) are added to the flask contents which are stirred at 100° C. for 15 minutes to dissolve the urea. The remaining half of the phosphorus pentoxide is then added, in portions, while holding the temperature at 100 to 110° C. When all of the phosphorus pentoxide has been thus added, the mixture is stirred for 1 hour more, while the temperature is held in the range between 100 and 110° C. The resulting reaction product is mixed with crushed ice and neutralized with aqua ammonia to have a pH between

5 and 8, yielding a hazy liquid with a solid content of about 50 wt. percent which is dilutable with water to provide faintly hazy solutions.

In this example, the reaction mixture has 1 atom of phosphorus supplied in the form of phosphoric acid and 3 atoms of phosphorus supplied in the form of phosphorus pentoxide, that is, a total of 4 atoms of phosphorus, per molecule of 2,3-dibromopropanol. The 2.44 gram-molecular weights of water (1.5 gram-molecular weights of free water and 0.94 gram-molecular weights of combined water) contained in the 85% phosphoric acid combined with the 1 gram-atomic weight of phosphorus contained in the phosphoric acid and with 2 of the gram-atomic weights of phosphorus supplied in the form of phosphorus pentoxide, to provide the desired ratio (2.44:3) of 0.8 molecule of water per atom of phosphorus in addition to the remaining 1 atom of phosphorus in the form of phosphorus pentoxide which is available for each molecule of 2,3-dibromopropanol.

#### EXAMPLE 5

218 grams of 2,3-dibromopropanol (1 gram-molecular weight) are disposed in a flask equipped with a stirrer and thermometer, and 71 grams of phosphorus pentoxide (containing 1 gram-atomic weight of phosphorus) are added thereto. The flask contents are stirred at 80 to 100° C. for 2 hours, and then 18 grams of water in the form of chopped ice (1 gram-molecular weight) are added thereto. Thereafter, over a period of 1 hour, 89 grams of phosphorus pentoxide are added to the flask contents followed by the addition of 18 grams of chopped ice (1 gram-molecular weight of water) and then by the gradual addition of a further 89 grams of phosphorus pentoxide over a period of 1 hour. The 178 grams of phosphorus pentoxide thus added contain an additional 2.5 gram-atomic weights of phosphorus. Thus, the reaction mixture contains 2 gram-molecular weights of water which, with respect to 2.5 of the gram-atomic weights of phosphorus provided in the form of phosphorus pentoxide, gives the desired 0.8 ratio of molecules of water to atoms of phosphorus, while 1 atom of phosphorus in the form of phosphorus pentoxide remains for each molecule of 2,3-dibromopropanol. Further, the ratio of total atoms of phosphorus per molecule of 2,3-dibromopropanol is 3.5:1.

After the final additions to the reaction mixture, the latter is stirred for 2 hours at 80 to 100° C., whereupon the reaction product is poured onto one-half its own weight of chopped ice and neutralized with sufficient concentrated aqua ammonia to provide a final product with a pH in the range between 5 and 8 and a solids content of approximately 50 wt. percent. Such final product is a clear solution with a faint yellow color.

#### EXAMPLE 6

218 grams of 2,3-dibromopropanol (1 gram-molecular weight) are mixed, for 1 hour at 80° C., with 932 grams of 105% polyphosphoric acid (containing 10 gram-atomic weights of phosphorus and approximately 12.3 gram-molecular weights of combined water). Then 384 grams of phosphorus pentoxide (containing about 5.4 gram-atomic weights of phosphorus) are added slowly to the reaction mixture while holding the temperature thereof between 80 and 100° C., whereby the 12.3 gram-molecular weights of water and the 15.4 gram-atomic weights of phosphorus in mixture result in the desired ratio of 0.8 molecule of water per atom of phosphorus. 180 grams of urea (3 gram-molecular weights) are added to the reaction mixture which is then further mixed for 1 hour at 100° C., followed by the addition of 142 grams of phosphorus pentoxide (containing 2 gram-atomic weights of phosphorus) and stirring of the final reaction mixture for 2 hours at 80 to 100° C. It will be seen that the final reaction mixture contains a total of 17.4 atoms of phosphorus per molecule of 2,3-dibromopropanol, with 2

atoms of phosphorus in the form of phosphorus pentoxide being available for each molecule of 2,3-dibromopropanol in addition to the atoms of phosphorus required for the desired ratio of 0.8 molecule of water per atom of phosphorus.

The reaction product is poured onto one-half its own weight of crushed ice and neutralized with concentrated aqua ammonia sufficient to provide a solution with a pH between 5 and 8 and a solids content of about 50 wt. percent. Such solution is a substantially clear liquid, which is further dilutable with water to yield clear solutions.

#### EXAMPLE 7

218 grams of 2,3-dibromopropanol (1 gram-molecular weight) are mixed, for 1 hour at 80° C., with 1978 grams of 115% polyphosphoric acid (containing 23 gram-atomic weights of phosphorus and 0.8 molecule of combined water per atom of phosphorus). 180 grams of urea (3 gram-molecular weights) are added to the mixture which is then stirred for 1 hour at 100° C., whereupon, 142 grams of phosphorus pentoxide (containing 2 gram-atomic weights of phosphorus) are added and the final reaction mixture is stirred for 2 hours at 80 to 100° C.

The reaction mixture here described has a total of 25 atoms of phosphorus per molecule of 2,3-dibromopropanol, 2 atoms of phosphorus in the form of phosphorus pentoxide per molecule of 2,3-dibromopropanol in addition to the atoms of phosphorus required for the 0.8 ratio of water molecules to phosphorus atoms, and a urea content that is less than 1 molecule thereof per each two atoms of total phosphorus.

The reaction product of the above mixture is poured on crushed ice and neutralized with concentrated aqua ammonia to a pH of 5 to 8 to yield a substantially clear solution containing approximately 50 wt. percent solids and which is further dilutable with water.

#### EXAMPLE 8

A woven cotton fabric weighing 4 ounces per yard is impregnated with a water diluted solution of the product of Example 1 and then dried at 240° F. The concentration of the impregnating solution is selected so as to result in an 11.0 wt. percent add-on with respect to the dried fabric. The treated fabric feels soft and there is very little change in its color.

A sample of the fabric thus treated is subjected to the flame retardancy test specified as AATCC #34-1966, in which a fabric specimen 10 inches long is held vertically in a metal frame which exposes a 2 inch width of the fabric. The lower edge of the exposed width of fabric is ignited by a yellow Bunsen burner flame 1.5 inches long which is held in contact with the fabric for a 12 second ignition period. The char-length of the treated fabric, measured upwardly from its lower edge, is less than 3 inches, and there is no after flame when the igniting flame is removed from the fabric at the end of the stated ignition period.

Results similar to those indicated above are attained when the fabric is similarly treated with the product of Example 5.

#### EXAMPLE 9

A knitted fabric consisting of 10% spandex fiber and 90% nylon, by weight, is treated, as in Example 8, with an aqueous solution containing equal parts, by weight, of ammonium phosphate and of the solids content of the product of Example 1 to provide a total dry add-on of 23 wt. percent. The treated fabric has only a slightly stiffer feel than the untreated fabric, and shows no crystallization of the treating substances which are not dislodged from the fabric by shaking or rubbing. When the fabric treated with the combination of ammonium phosphate and the product of Example 1, as here described, is subjected to the AATCC #34-1966 flame retardancy test, there is only a 3.5 inch char length and no after flame.

As distinguished from the foregoing, when a specimen of the same fabric is treated with a solution of ammonium phosphate alone and dried so as to have a dry add-on of 23 wt. percent, the treated fabric is stiff and has a powdery deposit thereon which is dislodged by shaking or rubbing. Further, the fabric treated with ammonium phosphate alone so as to have a dry add-on of 23 wt. percent burns along its entire length when subjected to the AATCC #34-1966 flame retardancy test.

#### EXAMPLE 10

A woven fabric composed of equal parts, by weight, of secondary cellulose acetate fibers and viscose rayon fibers, is treated with an aqueous solution of the product of Example 2 and then dried so as to have a dry add-on of 13 wt. percent of the solids in such product. The thus treated fabric does not exhibit any crystallization of the treating solids thereon and has a substantially unchanged feel. When the treated fabric is subjected to the described AATCC #34-1966 flame retardancy test, a 4.0 inch char length is obtained.

Reducing the dry add-on of the product of Example 2 to 10 wt. percent, the thus treated fabric of secondary cellulose and viscose rayon has a char length of 5.5 inches.

In contrast to the foregoing, the same fabric requires an 18 wt. percent dry add-on of ammonium phosphate to exhibit a char length of 4.0 inches, and such add-on of ammonium phosphate results in undesirable stiffness of the treated fabric and a powdery appearance due to crystallization.

#### EXAMPLE 11

An aqueous solution of the product of Example 2 is applied to a knitted fabric composed of 10% spandex and 90% nylon so as to provide, upon drying of the treated fabric, a 22 wt. percent dry add-on of the solids in the product of Example 2. The treated knitted fabric, when subjected to the AATCC #34-1966 flame retardancy test, has a char length of 2.5 inches and exhibits no after flame. Further, the fabric with a 22 wt. percent add-on of the product according to this invention exhibits very little stiffening and no crystallization.

As contrasted with the foregoing, the same 10% spandex and 90% nylon knitted fabric requires a 28 wt. percent dry add-on of ammonium phosphate in order to exhibit a char length of 5.0 inches in the identified flame retardancy test, and even then has an after flame of 30 seconds duration. Further, the fabric with a 28 wt. percent dry add-on of ammonium phosphate exhibits substantial stiffening and a powdery surface due to crystallization.

#### EXAMPLE 12

An aqueous solution of the product of Example 2 is applied to a 90% triacetate-10% nylon fabric which is then dried to provide a 3.5 wt. percent dry add-on of the solids in the product of Example 2. A surface of the treated fabric is napped. A specimen of the napped treated fabric is held in a plane at 45° to the horizontal with the napped surface facing upwardly and, when such napped surface is ignited, at its center, by a match flame, no surface flash occurs. However, when the same napped fabric, but without the treatment thereof with the flame retardant according to this invention, is subjected to the same test, the ignition at the center of the napped surface results in an almost instantaneous surface flash of the flame to all parts of the specimen. Thus, although the mentioned fabric having only a 3.5 wt. percent add-on of the product of Example 2 will burn its entire length when subjected to the vertical AATCC #34-1966 test, such small add-ons are nevertheless effective as flame-retardants, particularly where it is only necessary to eliminate the hazard of surface flash.

## EXAMPLE 13

A woven fabric composed of 65 wt. percent polyester and 35 wt. percent cotton is impregnated with an aqueous solution containing 3 parts, by weight, of ammonium sulfamate and 1 part, by weight, of the solids in the product of Example 2, and then dried so as to have a dry add-on of 26 wt. percent. The treated fabric is soft and exhibits a 3.5 inch char length in the AATCC #34-1966 vertical flame retardancy test.

As contrasted with the foregoing, the same fabric, when treated with a solution of ammonium sulfamate alone so as to have a 26 wt. percent dry add-on of the latter, burns along its entire length when subjected to the identified vertical flame retardancy test.

## EXAMPLE 14

The tests of Example 13 are repeated with respect to a rayon non-woven fabric containing 20 wt. percent of acrylic resin binder. Such fabric having a 20 wt. percent dry add-on of ammonium sulfamate alone burns its entire length upon being subjected to the AATCC #34-1966 test, but the same fabric having a 20 wt. percent dry add-on of the mixture of ammonium sulfamate and the solids of the product of Example 2, in the 3:1 ratio, has a char length of 3.0 inches.

## EXAMPLE 15

A woven cotton fabric weighing 4 ounces per yard is treated with ammonium sulfate alone so as to have an 11 wt. percent dry add-on thereof. When such treated fabric is subjected to the AATCC #34-1966 test, it exhibits an erratic flammability behavior. Thus, with a 12 second period of ignition by a Bunsen burner flame, which is the standard ignition period, the fabric has a 4.0 inch char length. However, if the ignition period is reduced to 5 seconds, the fabric burns for its entire length.

As contrasted with the foregoing, the same fabric provided with an 11 wt. percent dry add-on of a mixture of ammonium sulfate and of the solids of Example 2, in a 5:1 weight ratio, exhibits a 2.5 inch char length, regardless of the duration of the ignition period, in the standard vertical test. Further, the latter treatment provides the fabric with a softer and smoother feel than the treatment with ammonium sulfate alone. This demonstrates how an inexpensive and relatively ineffective flame retardant salt, such as ammonium sulfate, can have its effectiveness and reliability substantially upgraded by the addition thereto of as little as 20 wt. percent of a product according to this invention.

## EXAMPLE 16

The same fabric as in Example 15 is treated with an aqueous solution of ammonium chloride alone so as to have a 16 wt. percent dry add-on of the latter. Such add-on of ammonium chloride makes the fabric quite stiff and the treated fabric burns its entire length when subjected to the AATCC #34-1966 test.

On the other hand, the same 16 wt. percent dry add-on of a mixture of ammonium chloride and the solids of the product from Example 2, in a 4:3 weight ratio, imparts to the treated fabric a feel that is only slightly stiffer than the untreated fabric. Further, the fabric treated with the defined mixture exhibits a char length of 3.5 inches in the standard test.

## EXAMPLE 17

An aqueous solution of the product of Example 3 is applied to a woven fabric composed of equal parts, by weight, of secondary cellulose acetate fibers and viscose rayon fibers so as to provide the dried fabric with a 13 wt. percent dry add-on of the solids. The treated fabric exhibits some increase in its stiffness but no crystallization. When the treated fabric is subjected to the AATCC #34-1966 test, a 3.5 inch char length is obtained.

Results similar to those indicated above are obtained when the fabric is similarly treated with the product of Example 6.

The application of the product of Example 7 to the fabric so as to obtain a 13 wt. percent dry add-on, as indicated above, results in the attainment of similar flame retardancy, with a tendency to increase the stiffness of the treated fabric. Further, when the product of Example 7 is applied to fabrics containing hydrophobic fibers, such as nylon, there is some tendency for the finish to crystallize on the surfaces of the non-water absorbent fibers, but this tendency is much less than the crystallization experienced with the same add-ons of inorganic flame-retardant salts, such as ammonium phosphate.

15

## EXAMPLE 18

A knit fabric composed of 90 wt. percent triacetate and 10 wt. percent nylon is impregnated with an aqueous solution of ammonium bromide and dried to provide a 23 wt. percent dry add-on of the ammonium bromide. Although the fabric thus treated with ammonium bromide has a char length of 4.8 inches when subjected to the AATCC #34-1966 vertical test, the treated fabric is stiff and has a whitish crusty appearance, due to crystallization, that makes the treated fabric unacceptable for commercial use. However, when the same fabric is treated with an aqueous solution of ammonium bromide and the product of Example 3 in the weight ratio of 9:1, and the wt. percent dry add-on of the mixture of solids is 23 wt. percent, the treated fabric does not exhibit a white, crusty appearance and, moreover, its char length in the standard vertical test is only 4.0 inches. Further, the fabric is not unacceptably stiff. Thus, it will be seen that the addition of relatively small proportions of a flame retardant according to this invention to an inorganic salt, such as ammonium bromide, can correct undesirable characteristics of the latter as an inexpensive flame retardant.

## EXAMPLE 19

40 Aqueous solutions of the product of Example 4 are applied to woven cotton fabrics of various weights and constructions, and are found to make such fabrics fire resistant according to the AATCC #34-1966 test with dry add-ons of the solids ranging from 9 to 13 wt. percent. 45 The lower add-ons of the fire retardant are effective to impart fire resistance, that is, to prevent burning of the fabric specimen along its entire length, in the case of the relatively heavier fabrics, whereas the larger concentrations (13 wt. percent add-on) are required for the lighter fabrics, such as, 4 ounce per yard fabrics.

40 It should be noted that the previously mentioned ammonium salt of 2,3-dibromopropylphosphoric ester is only sparingly soluble in water and is a costly compound in comparison with such substances as ammonium phosphate and ammonium sulfamate. The foregoing is true because the relatively costly 2,3-dibromopropanol is a major proportion of the mentioned compound. However, with the products according to this invention, the weight proportion of dibromopropanol can be greatly reduced, as is apparent from the foregoing examples, while retaining most of the advantages of the unmodified ester. Further, the products according to this invention may be admixed with inorganic flame retardant salts, to improve the properties of such inexpensive salts as in certain of the examples. 60 However, it is to be understood that the products of this invention are not mere mixtures of the normal dibromopropylphosphoric ester with ammonium phosphate or ammonium polyphosphate, although it is possible that minor amounts of these latter salts may be present in the reaction products due to side reactions. An indication of the fact that the reaction products according to the invention are true chemical compounds and not mere mixtures is found in their solubility in water which is far higher than that of the unmodified dibromopropylphosphoric ester. This enhanced solubility in water, which in-

creases with the proportion of phosphorus in the compound, I believe to be due to the presence of a plurality of polyphosphoric acidic hydroxyl groups in the molecule. As the number of such groups increases, the water-solubility of the entire molecule increases, particularly in the form of the ammonium salt thereof.

Having described the invention with particular reference to precise examples thereof, it is to be understood that the invention is not limited to those examples, and that various modifications and changes may be made by one skilled in the art without departing from the scope or spirit of the invention.

What is claimed is:

1. The reaction product obtained by mixing, at a temperature in the range from approximately 80° C. to approximately 110° C., 2,3-dibromopropanol, phosphorus pentoxide in an amount sufficient to provide therein from 1 to 2 atoms of phosphorus per molecule of said 2,3-dibromopropanol, at least one additional phosphorus-containing substance selected from the group consisting of phosphorus pentoxide, phosphoric acid and polyphosphoric acid in an amount to provide with the first-mentioned phosphorus pentoxide a total of approximately from 3 to 25 atoms of phosphorus per molecule of said 2,3-dibromopropanol, and from 0 to approximately 0.8 molecule of free water for each atom of phosphorus in said additional phosphorus-containing substance so as to provide with any combined water in the latter a total water content of approximately 0.8 molecule of water for each phosphorus atom in said additional phosphorus-containing substance.

2. The reaction product according to claim 1, in which said mixture further contains urea in an amount sufficient to provide a maximum of 1 molecule of urea for each 2 atoms of phosphorus in said total atoms of phosphorus.

3. A water-soluble flame retardant consisting essentially of the reaction product of claim 2 dissolved in water and neutralized with ammonia to a pH in the range from approximately 5 to 8.

4. A flame retardant according to claim 3, in which the amount of water in which said reaction product is dissolved is sufficient to provide a solids content therein of from 50 to 55 wt. percent.

5. A water-soluble flame retardant consisting essentially of an aqueous solution of the reaction product obtained by mixing, at a temperature in the range from approximately 80° C. to approximately 110° C., 2,3-dibromopropanol, sufficient 115% polyphosphoric acid to provide 2 atoms of phosphorus per molecule of 2,3-dibromopropanol, and sufficient phosphorus pentoxide to provide 1 atom of phosphorus per molecule of 2,3-dibromopropanol, and sufficient ammonia in said solution to provide a pH thereof in the range from 5 to 8.

6. A water-soluble flame retardant consisting essentially of an aqueous solution of the reaction product obtained

40

45

50

55

by mixing, at a temperature in the range from approximately 80° C. to approximately 110° C., 2,3-dibromopropanol, sufficient 115% polyphosphoric acid to provide 6 atoms of phosphorus per molecule of 2,3-dibromopropanol, sufficient urea to provide 3 molecules thereof per molecule of 2,3-dibromopropanol and sufficient phosphorus pentoxide to provide 2 atoms of phosphorus therein per molecule of 2,3-dibromopropanol, and sufficient ammonia in said solution to provide a pH thereof in the range from 5 to 8.

7. A water-soluble flame retardant consisting essentially of an aqueous solution of the reaction product obtained by mixing, at a temperature in the range from approximately 80° C. to approximately 110° C., 2,3-dibromopropanol, sufficient 115% polyphosphoric acid to provide 18 atoms of phosphorus therein per molecule of said 2,3-dibromopropanol, 2-molecules of urea per molecule of said 2,3-dibromopropanol and sufficient phosphorus pentoxide to provide 2 atoms of phosphorus therein per molecule of said 2,3-dibromopropanol, and sufficient ammonia in said solution to provide a pH thereof in the range from 5 to 8.

8. A water-soluble flame retardant consisting essentially of an aqueous solution of the reaction product obtained by mixing, at a temperature in the range from approximately 80° C. to approximately 110° C., 2,3-dibromopropanol, sufficient 85% phosphoric acid to provide 1 atom of phosphorus therein per molecule of said 2,3-dibromopropanol, sufficient urea to provide 2 molecules thereof per molecule of said 2,3-dibromopropanol and sufficient phosphorus pentoxide to provide 3 atoms of phosphorus therein per molecule of said 2,3-dibromopropanol, and sufficient ammonia in said solution to provide a pH thereof in the range from 5 to 8.

9. A water-soluble flame retardant consisting essentially of an aqueous solution of the reaction product obtained by mixing, at a temperature in the range from approximately 80° C. to approximately 110° C., 2,3-dibromopropanol, sufficient phosphorus pentoxide to provide 3.5 atoms of phosphorus therein per molecule of said 2,3-dibromopropanol and sufficient free water to provide 2 molecules thereof per molecule of said 2,3-dibromopropanol, and sufficient ammonia in said solution to provide a pH thereof in the range from 5 to 8.

#### References Cited

#### UNITED STATES PATENTS

3,283,013 11/1966 Rimmer \_\_\_\_\_ 260—933 X

CHARLES B. PARKER, Primary Examiner

A. H. SUTTO, Assistant Examiner

U.S. CL. X.R.

106—15 FP; 117—137; 260—924, 933, 980